

# UNITED STATES PATENT OFFICE.

FRANK E. BURGESS, OF COLUMBIAVILLE, MICHIGAN.

## PROCESS FOR BLEACHING AND TREATING FLAX FIBERS.

1,034,195.

Specification of Letters Patent. Patented July 30, 1912.

No Drawing.

Application filed March 30, 1912. Serial No. 687,458.

*To all whom it may concern:*

Be it known that I, FRANK E. BURGESS, a citizen of the United States, residing at Columbiaville, in the county of Lapeer and

5 State of Michigan, have invented new and useful Improvements in Processes for Bleaching and Treating Flax Fibers, of which the following is a specification.

This invention relates to processes for 10 treating and bleaching flax fibers and the principal object of the invention is to not only bleach the flax or linen in its raw state to a perfect white but to also destroy the woody substance found in the raw flax without injuring the fine fiber.

15 The process is adapted to leave the stock in condition so that it can be immediately manufactured into any textile article.

Heretofore, the process of removing the 20 woody substance from the fine fiber and the bleaching process has been formed by two distinct operations, the first consisting and allowing the fiber to rot on the ground or to rot in vats and then bleaching the stock.

25 I accomplish the same results by practically one operation, and, specifically speaking, the invention consists in treating the raw flax to a caustic bath and then bleaching the stock in a bath of sulfite of sodium.

30 The method of carrying out the process is as follows: First, the material is boiled in water for a predetermined time to soften the fibers so that the chemicals which are applied thereto in the following steps may have rapid and direct action. The surplus water is then removed from the stock by means of a hydro-extractor or any other suitable manner and the mass then subjected 35 to a bath charged with caustic soda or caustic potash of a specific gravity of say 50°

to 60° Twaddell, at the temperature of 100° Fahrenheit or under without drying. The mass is then washed in water and subjected to a bath charged with sulfite of sodium of a sufficient strength and at a sufficient temperature to properly bleach the fiber. It has been proposed to use sodium carbid, sulfuric acid, carbon dioxid, and water to bleach the flax fibers but by this method 45 only a three-quarter bleach may be produced and it is essential that the stock be bleached pure white for in that state it can be dyed in any bright or dull color or even manufactured without dyeing, in which case the result may be a perfectly white article. With 50 a three-quarter bleach, this is impossible.

It is to be understood that the strength of the potash or soda bath or the strength and temperature of the bath of sulfite of sodium 55 may be varied without deviating from my invention as good results have been obtained in baths of varying strengths and temperatures.

What is claimed is:—

The process of treating flax fibers which 60 consists in boiling the material in water, removing the surplus water, subjecting the material to a bath charged with caustic potash or caustic soda of a specific gravity of approximately 50° or 60° Twaddell at a 65 temperature of approximately 100° Fahrenheit, washing the treated material, and subjecting the same to a bath charged with 70 sulfite of sodium.

In testimony whereof I affix my signature 75 in presence of two witnesses.

FRANK E. BURGESS.

Witnesses:

B. E. McDERMID,  
R. C. WIXSON.